

Patented July 22, 1924.

1,502,101

# UNITED STATES PATENT OFFICE.

CHARLES A. HUTTINGER, OF LAKWOOD, OHIO, ASSIGNOR TO THE ACME ARTIFICIAL SILK COMPANY, OF CLEVELAND, OHIO, A CORPORATION OF OHIO.

## PROCESS OF MANUFACTURING VISCOSE.

No Drawing.

Application filed June 28, 1922. Serial No. 571,567.

To all whom it may concern:

Be it known that I, CHARLES A. HUTTINGER, a citizen of the United States, resident of Lakewood, county of Cuyahoga, and 5 State of Ohio, have invented new and useful Improvements in Processes of Manufacturing Viscose, of which the following is a specification, the principle of the invention being herein explained, and the best mode in which 10 I have contemplated applying that principle so as to distinguish it from other inventions.

The subject matter of this application has been divided out of my pending application, 15 Serial No. 303,776, filed June 12, 1919.

My invention relates to processes of manufacturing viscose. The purpose of the invention is to compound a viscose solution effective in producing lustrous threads of 20 the character described and claimed in my U. S. Letters Patent No. 1,425,654. By the improvements herein described and claimed I am enabled to make a viscose solution suitable for producing a lustrous thread of the 25 necessary qualities as regards its luster, strength and elasticity, without the necessity of using any free acid in the precipitating bath and without the necessity of heating the latter above the usual working room 30 temperature. I accomplish this object both by the proportions of the ingredients which I utilize in making my viscose solution and in my methods of compounding same.

The following description sets forth in 35 detail certain steps illustrating the method of carrying out my invention, such described steps constituting, however, but one of the various ways in which the principle of the invention may be utilized.

In carrying out my improved process, I 40 cut up a certain amount of wood pulp, one kilogram for instance, and then saturate the same with sodium hydroxide. The saturation is effected by a water solution of sodium hydroxide of substantially 1.17 specific gravity. The amount of sodium hydroxide which 45 I use, for the stated amount of wood pulp, is substantially 515 grams, and the amount of water utilized in making a solution of the specific gravity noted is substantially 2918 50 grams, which is a 15 per cent solution of sodium hydroxide. The treatment of the wood pulp with this sodium hydroxide solution continues for from one to five hours, 55 preferably about one and a half hours. I

then subject the wood pulp and sodium hydroxide water solution to great pressure, by means of a hydraulic press when treating comparatively large amounts, or by means of a screw press for small quantities, so that 60 the material remaining on the press, i. e., the alkali cellulose, amounts to substantially 3 kilograms, when using the various amounts stated. Of these 3 kilograms, substantially 13.5 per cent is alkali, including the small 65 amount which is free, as well as that which has combined, substantially 27 per cent is cellulose, and the remainder, 59.5 per cent, is water. I grind up these 3 kilograms of alkali cellulose remaining on the press, this 70 alkali cellulose being a crumby material. I then subject the same to the action of substantially 325 grams of carbon bisulphide for about two hours. I then add water of substantially fifteen (15) times the amount 75 of wood pulp originally utilized, or, as exactly as I have determined, 15.023 kilograms of water, the mixture being allowed to stand for substantially three hours. This 80 comparatively large amount of water will dissolve some of the small amount of free sodium hydroxide in the alkali cellulose-carbon bisulphide mixture, so that the water is slightly alkaline. The resultant mixture is filtered 85 during an aging period of about five days.

The viscose solution compounded as above can be spun into a lustrous thread, having all the desirable qualities in the proper degree, in a precipitating bath containing no free acid and used at substantially the usual 90 working room temperature, as described and claimed in said Patent No. 1,425,654. My explanation of my ability to thus secure a satisfactory thread, under these conditions, is that my method of compounding the viscose solution results in a saturation of the wood pulp with sodium hydroxide without there being present in the solution thereafter a high percentage of free sodium hydroxide, which free sodium hydroxide must necessarily be neutralized out of the solution to leave the cellulose for the thread. This neutralization has been effected heretofore by the acid used. Thus, the lack of 95 surplus hydroxide in my method obviates the necessity of free acid for neutralizing such sodium hydroxide.

What I claim is:

1. In processes of manufacturing viscose, the steps which consist, in saturating wood

- pulp with a water solution of sodium hydroxide of substantially a specific gravity of 1.17, and subjecting the mixture of said wood pulp and said solution to great pressure so that the resultant alkali cellulose will equal substantially three times the amount of wood pulp utilized, and of which the cellulose will comprise substantially 27 per cent; adding carbon bisulphide to the alkali cellulose of substantially one-third the amount of the original wood pulp utilized; adding a comparatively large amount of water; and filtering.
2. In processes of manufacturing viscose, the steps which consist, in saturating wood pulp with a water solution of sodium hydroxide of substantially a specific gravity of 1.17, and subjecting the mixture of said wood pulp and said solution to great pressure so that the resultant alkali cellulose will equal substantially three times the amount of wood pulp utilized, and of which the cellulose will comprise substantially 27 per cent; grinding said alkali cellulose; adding carbon bisulphide thereto of substantially

one-third the amount of the wood pulp originally utilized; adding water of substantially fifteen times the amount of wood pulp originally utilized; and filtering.

3. In processes of manufacturing viscose, the steps which consist, in saturating one kilo of wood pulp with a sodium hydroxide water solution consisting of substantially 515 grams of sodium hydroxide and 2918 grams of water, said treatment continuing for substantially one and a half hours; subjecting the mixture to great pressure, so that the resultant alkali cellulose will equal substantially 3 kilograms, of which 13.5 per cent is combined and free sodium hydroxide and 27 per cent is cellulose; grinding up the resultant alkali cellulose, and then subjecting the same for substantially two hours to the action of 325 grams of carbon bisulphide; adding substantially 15 kilograms of water; and filtering and aging for substantially 5 days.

Signed by me, this 6th day of June, 1922.

CHARLES A. HUTTINGER.